

## UNITED STATES PATENT OFFICE

2,292,795

## FOUNDRY PARTING

Marion W. Pitner, Chicago, Ill., assignor, by  
mesne assignments, to Delta Oil Products Com-  
pany, a corporation of Wisconsin

No Drawing. Application August 2, 1940,  
Serial No. 350,082

2 Claims. (Cl. 22—189)

My invention relates to improvements in foundry partings and the process of manufacturing such partings.

It is the primary object of the invention to provide a novel and commercially satisfactory foundry parting material and process of manufacture thereof.

More specifically, it is the object of the present invention first, to avoid the production of a foundry parting having an unpleasant odor, and secondly, to employ chemicals economically to render water repellent a flour-like material which is otherwise entirely satisfactory for foundry parting purposes. As an illustration and example of my process and the product resulting therefrom, I shall describe the application of the process to walnut shell flour to impart thereto the necessary water repellency. Walnut shell flour of a fineness between 100 mesh and 300 mesh would, in its untreated state, be ideally suited to foundry parting purposes but for the fact that it is wettable. Previous attempts to make nutshell flour unwettable have not been commercially successful due in part to spontaneous combustion and in part to objectionable odors resulting from the use of soaps and waxes, and due in part to the absorption of chemicals by the flour with a consequent abnormally high consumption of the chemicals used for water repellency and also to undesirable resistance of the resulting product to passage through the dusting bag used in the foundry.

Specifically, it is my purpose to avoid the above mentioned difficulties.

My process may be carried out in any container wherein the contents may be heated and mixed. The following is an example of the proportions which may be used in the practice of my process.

To 35 gallons of cold water I add 100 pounds of walnut shell flour, 8.5 pounds of aluminum sulphate, and 3 pounds of sodium aluminate. After these materials have been mixed I add an additional 30 gallons of cold water and then raise the entire mixture to the boiling point and boil for five minutes. The product of this treatment is filtered and washed with three successive charges of 30 gallons each of boiling water, after which the product is dried in a vacuum drier.

It will be noted that the amount of chemicals used is relatively small. The weight of chemicals is only slightly greater than the amount of wax which might be used in a process employing waxes or fats as a waterproofing agent. Yet the

waxes or fats would impregnate the material and make it spontaneously combustible and malodorous in storage. By confining my process to the use of chemicals I avoid these objectionable results. Moreover, by mixing the aluminum sulphate and the sodium aluminate in the presence of the particles of flour, I form directly in the presence of the flour the aluminum oxide which is believed to be adsorbed superficially on the flour particles and to be responsible for their water repellent characteristics. The formation of aluminum oxide directly in the presence of the flour and with only a limited period of boiling, precludes absorption or impregnation of the chemicals into the particles of flour and thereby not only reduces the amount of chemicals which would otherwise be required, but also makes a product which is better-suited for use in the dusting bag of the foundry.

As a by-product of the production of aluminum hydroxide, which later breaks down into aluminum oxide above referred to, sodium sulphate is produced. This is washed from the product in the final stages of the treatment above described.

I have encountered certain walnut shell flour which would not satisfactorily respond to the foregoing treatment and required the addition of stearic acid. I have, however, discovered how stearic acid may be used in connection with the foregoing process and the foregoing chemicals in a manner which avoids impregnation or absorption of the particles of flour and also avoids the production of a product which would be either spontaneously combustible or malodorous. If it is necessary to use stearic acid, I practice my process as follows.

100 pounds of walnut shell flour and 8.5 pounds of aluminum sulphate are mixed with 40 gallons of cold water in one container. In a separate container  $\frac{3}{4}$  pound of sodium hydroxide and 3 pounds of stearic acid are mixed in 40 gallons of water at a temperature approximately 180° F. When the mixture in the second container is saponified I add thereto and mix therewith three pounds of dry sodium aluminate. The contents of the two containers are then combined and agitated to mix all of the ingredients with or without a brief period of heating as above described. The filtration and washing is then carried on as in my first process to wash away the sulphate by-product. The resulting product, even though neo-fat or stearic acid is included, is water repellent by reason of a coating adsorbed upon the particles, rather than impregnated

therein, and the particles have the same distinctive individuality and lack of mutual adhesion that is characteristic of the original product. They are water repellent. They are not subject to spontaneous combustion, and they have no objectionable odor.

The particles of flour are so fine that it is difficult to examine them adequately, but chemical and physical analysis both indicate that the desirable attributes of the product of this invention are attributable to the fact that the anhydrous aluminum oxide which provides the water repellent characteristic (and the stearic acid, if small amounts thereof are used in accordance with the second process herein disclosed) are 15 adsorbed superficially upon the particles instead of being absorbed or impregnated therein.

I claim:

1. The treatment of walnut shell flour to produce a foundry parting compound therefrom, 20 which treatment includes the separate prepara-

tion of batches of water in one of which there is aluminum sulphate and in the other of which there is sodium aluminate, the introduction of a neo-fat into one of said batches, the admixture of said batches in the presence of the flour requiring treatment whereby to deposit upon the particles of flour individual coatings containing aluminum oxide and neo-fat, and the washing and drying of the coated flour.

2. A process of treating walnut shell flour to render it suitable for use as a foundry parting compound, which process includes the mixing of the flour with water and aluminum sulphate in one container, the mixing of sodium hydroxide and stearic acid with water in another container, and the saponification of the materials in said second container, the admixture of sodium aluminate with the saponified material in the second container, and the subsequent admixture of the contents of the two containers.

MARION W. PITNER.